

# UNITED STATES PATENT OFFICE.

HEINRICH DRESLER, OF CREUZTHAL, GERMANY.

## MANUFACTURE OF BRICKS, SHAPED STONES, OR BLOCKS, TUBES, TILES, AND THE LIKE.

No. 903,062.

Specification of Letters Patent.

Patented Nov. 3, 1908.

Application filed September 23, 1908. Serial No. 454,353.

*To all whom it may concern:*

Be it known that I, HEINRICH DRESLER, director of the Cöln Müsener Bergwerks Oe-  
5 tien Verein, of Creuzthal, Westphalia, Ger-  
many, a subject of the German Emperor,  
and resident of Creuzthal, Westphalia, Ger-  
many, have invented a new and useful Im-  
proved Manufacture of Bricks, Shaped  
10 Stones, or Blocks, Tubes, Tiles, and the Like,  
of which the following is a specification.

Slag stones, or blocks hardened by means  
of carbonic acid, have been hitherto manu-  
factured from either water-granulated slag  
or ground slag solidified in the open air.

15 This invention relates to the manufacture  
of bricks, stones, pipes, tiles and the like  
from slag with the action of carbonic acid,  
or gases containing carbonic acid, on the  
molded or shaped articles, with or without  
20 addition of lime, the novelty of this process  
being that the manufacture of the moldings  
is effected not, as hitherto, from a single slag  
material, but from a mixture of slags pre-  
pared in different manners. Thus, for in-  
25 stance, slag granulated by means of water, is  
mixed with slag solidified in the open air and  
reduced or ground or in a decomposed  
state. By slag solidified in the open air is  
meant slag which is cooled in the air from  
30 the hot liquid state and solidified. In prac-  
tice it is also called "block" or "piece"  
slag.

In the following description the aforemen-  
tioned mixture is moistened with water in  
35 the manner usual in the case of slag blocks  
or moldings, and compressed into molds or  
forms which are then exposed to the action  
of carbonic acid under pressure. This pro-  
cess has the advantage over similar well  
40 known processes that the weight of the  
blocks etc. can be considerably reduced, with-  
out affecting the required strength of the  
same. The blocks or products obtained are  
of beautiful appearance as the slag grains  
45 and the slag powder appear to have melted  
or blended therein into one mass. For in-  
creasing the strength, it may be advisable in  
certain cases to add a small percentage of  
lime. The experiments of the applicants  
50 have shown however that a mixture of 50%  
of slag powder or meal, and 50% of slag  
sand, even without addition of lime, gives a  
product which can resist a pressure of over  
4500 pounds per square centimeter. This  
55 strength is sufficient for all purposes, and  
the reduction of weight referred to enables

the blocks etc. to be shipped to greater dis-  
tances than would be economically possible  
with stones made of slag solidified in the air,  
alone. As moreover the grinding of slag is 60  
more expensive than mixing and as with the  
same output of blocks the grinding is re-  
duced by the process according to this inven-  
tion, the cost of manufacture according to  
this process is considerably reduced, which 65  
means an important technical advantage.

The blocks prepared by the new process  
are porous, which, without affecting their  
strength, has the advantage that the mortar  
adheres well to their surface. Moldings 70  
which are made only from air-solidified slag,  
easily crack during compression, and on the  
removal of the press die adhere to the die, so  
that a great deal of waste is caused. If,  
however, a mixture of slag is used, according 75  
to this invention, the compression of the  
moldings takes place easily and without any  
waste. The hardening in vessels by car-  
bonic acid requires by this invention much  
less time, and, owing to the greater porosity, 80  
the acid penetrates deeper into the articles.  
The greater porosity of the blocks obtained  
by the process according to this invention,  
has the further advantage that the blocks  
dry more quickly, and thus buildings are 85  
rendered more healthy.

The process is preferably carried out in  
such manner that the two kinds of slag are  
mixed together, and the moldings are pre-  
pared from the said mixture without the use 90  
of any binding material. They are intro-  
duced then into an air tight closed tank, into  
which carbonic acid is admitted, and are  
thus caused to harden. In order to increase  
the action of the carbonic acid to a still 95  
greater extent, the tank in which the harden-  
ing takes place, is first entirely or partly  
pumped free from air after the introduction  
of the moldings, and before the admission of  
100 the carbonic acid. Gases containing car-  
bonic acid could however be also passed  
through the vessel which is then closed, a  
partial vacuum being automatically pro-  
duced by the absorption of the carbonic acid.

### Claims.

1. The process of manufacturing bricks  
and similar articles, which consists in mixing  
water granulated slag with ground slag that  
has been solidified in the open air, molding  
the mixture, and subjecting the molded prod-  
uct to the action of carbonic acid gas under  
pressure for the purpose of acting on any

105

110

free lime that may be present, substantially as described.

2. A composition of matter forming bricks and similar articles, consisting of a mixture of slag solidified in the open air and pulverized, and of slag granulated in water, molded together and hardened under pressure of carbonic acid gas, substantially as described.

3. A composition of matter forming bricks and similar articles, consisting of a mixture of slag solidified in the open air and pulverized and of slag granulated in

water, molded together in substantially equal parts and hardened by carbonic acid gas, substantially as described.

In testimony, that I claim the foregoing as my invention, I have signed my name in presence of two witnesses, this 9th day of September 1908.

HEINRICH DRESLER.

Witnesses:

Louis VANDORN,  
H. STELZER.